

## UNITED STATES PATENT OFFICE

1,968,855

## COLORING OF TEXTILE MATERIALS

George Rivat, Lyon, France, assignor to Celanese Corporation of America, a corporation of Delaware

No Drawing. Application February 20, 1931,  
Serial No. 517,313

9 Claims. (Cl. 8—5)

This invention relates to the coloring of textile materials containing cellulose acetate or other organic derivatives of cellulose in a very economical and expeditious manner.

5 An object of my invention is to color textile materials comprising organic derivative of cellulose yarn by a method that is very economical and which produces excellent results. A further object of my invention is to color cellulose acetate material by a process employing dyestuffs that have little or no affinity for cellulose acetate material when applied in the ordinary manner. Still another object of my invention is to print fabrics by applying the dyestuff in such a manner 15 that the necessity of steaming is obviated. Other objects of my invention will appear from the following detailed description.

I have found that if dyestuffs are applied to textile materials containing organic derivatives 20 of cellulose in the presence of a relatively large amount of volatile organic liquid of a relatively high boiling point, which liquid exerts at least a softening action on the organic derivative of cellulose, many new and startling results are obtained. In the first place, by this method, many dyestuffs of low cost, which have no affinity for the organic derivative of cellulose when applied in the ordinary manner, may be used to obtain bright colors which do not tend to rub. Secondly, when the method is employed for printing, mere drying at an elevated temperature below 30 100° C. is sufficient to fix the dye, and thus the use of the relatively expensive ager or cotton steamer for fixing by steaming is not required. Thirdly, brilliant colors may be obtained with the use of very small quantities of dyestuff. Furthermore if a delustered fabric is printed in accordance with this invention, the parts printed not only become colored, but also assume a bright 35 lustre.

In accordance with my invention I color fabrics containing organic derivatives of cellulose by applying thereto a composition containing a suitable dyestuff and a volatile organic liquid having a 40 boiling point above 100° C. that has at least a softening action on the organic derivative of cellulose.

The textile material to be treated may be in the form of a fabric containing yarns of organic derivatives of cellulose such as organic esters of cellulose or cellulose ethers. Examples of organic esters of cellulose are cellulose acetate, cellulose formate, cellulose propionate and cellulose butyrate, while examples of cellulose ethers 45 are ethyl cellulose, methyl cellulose and benzyl cellulose. The fabric may be a mixed fabric containing yarns of organic derivatives of cellulose and yarns of other fibres such as cotton, reconstituted cellulose, natural silk, wool, etc. Some of 50 the dyestuffs that may be used have no affinity

for the said other fibres, and thus differential color effects may be obtained.

The dyestuff may be applied locally in the form of a paste by printing or by spraying or brushing through stencils on to the fabric.

The composition containing the dye, as stated, contains a volatile organic liquid which has a boiling point above 100° C. and is a solvent for or acts to soften the organic derivative of cellulose. Such organic liquid is preferably miscible with 70 water. Examples of suitable liquids in the case of the treatment of cellulose acetate material are ethyl lactate, diacetone alcohol, and the acetate of mono ethyl ether of ethylene glycol. A suitable amount of organic liquid is used, in the case of 75 ethyl lactate this amount being 200 to 400 cc. per litre of composition.

Dyestuffs of various classes may be employed. This may be the indigosols, the basic dyestuffs and certain vat dyestuffs. A remarkable feature of 80 this invention is that the acid dyes, which have little or no affinity for cellulose acetate material when applied in the ordinary manner, produce excellent colorations when employed in this invention.

After the application of the dyestuff composition, the fabric may be given a simple drying at a temperature below 100° C., say 50 to 80° C., by passing over heated cans or through a heated atmosphere or in any other suitable manner. The 90 ordinary expensive steaming operation need not be employed, although its use is not excluded from the scope of this invention.

If a fabric containing delustered cellulose acetate yarn is printed with a paste made in accordance with this invention, and the fabric then dried, the locally treated parts become lustrous, thus producing lustrous colored effects against a matte background.

In order further to illustrate my invention, but 100 without being limited thereto, the following specific examples are given.

## Example I

A fabric consisting of cellulose acetate yarn is 105 printed with a paste made as follows:

|                                                       |            |       |
|-------------------------------------------------------|------------|-------|
| Dyestuff                                              | 10 to 40   | grams |
| Glyezine (thio diglycol)                              | 60 to 80   | grams |
| Water                                                 | 160        | grams |
| Ethyl lactate                                         | 200 to 600 | cc.   |
| Gumarabic thickener or colloresine (methyl cellulose) |            | 110   |
| other thickener (1:1)                                 | 400        | grams |

As dyestuff, the following may be used: 115

Formyl violet 5 B (color index No. 698)

Milling green (color index No. 667)

Chromacetine blue S (color index No. 884)

Acridine red (color index No. 770)

Rhoduline blue (color index No. 658) 120

- Chromazurine H. B. (color index No. 879)  
 Cupranil Brown B (color index No. 560)  
 Benzyl violet (color index No. 683)  
 Induline (color index No. 861)
- 5      Acridine orange (color index No. 788)  
 Acridine red P. S. (color index No. 740)  
 Alkali blue (color index No. 704)  
 Rhodamine 3 G. O. (color index No. 749)  
 Metanile yellow (color index No. 138)
- 10     Milling red (color index No. 344)  
 Polar red (color index No. 430)  
 Rhoduline yellow 6 G (color index No. 815)  
 Benzyl green (color index No. 667)
- If the fabric contains reconstituted cellulose or  
 15 cotton, differential color effects may be obtained  
 by using the following dyestuffs which have no  
 direct affinity for cotton or cellulose; polar red,  
 alkali blue, benzyl violet, milling green, benzyl  
 green or metanile yellow, etc.
- 20     After printing, the fabric is dried at 70 to 75° C.  
 for sufficient time to permit the vaporization of  
 the ethyl lactate. A short washing with luke  
 warm water then follows, after which the fabric  
 25 is soaped at 50° C. for 3 to 5 minutes in a soap  
 solution containing 2 to 3 grams of soap per  
 litre. The fabric is finally rinsed in the ordinary  
 manner.
- Example II*
- 30     A fabric consisting of cellulose acetate yarn  
 is printed with the following paste:
- |                      | Grams      |
|----------------------|------------|
| Diphenyl black base  | 40 to 50   |
| Aniline              | 100 to 120 |
| 35     Ethyl lactate | 200        |
| Glacial acetic acid  | 120        |
| Water and thickener  | 530        |
- After printing with the above paste, the fabric  
 40 is rapidly dried at 60 to 70° C. and is passed into  
 a bath consisting of a solution having the following  
 composition:
- |                         | Grams |
|-------------------------|-------|
| Sodium bichromate       | 15    |
| 45     Water            | 950   |
| Sulfuric acid of 66° Bé | 35    |
- The fabric is allowed to remain in this bichromate  
 50 bath at 15° to 20° C. for 2 minutes, is then  
 rinsed in cold water, treated in a bath containing  
 a cold solution of sodium carbonate of 5 grams  
 per litre for 1 minute, then scoured in a soap bath  
 at 80° C. for 5 minutes and finally washed.
- The fabric is dyed a black color which is very  
 55 bright and fast to rubbing.
- It is to be understood that the foregoing detailed  
 description is given merely by way of illustration  
 and that many variations may be made therein without departing from the spirit of my  
 60 invention.
- Having described my invention, what I claim  
 and desire to secure by Letters Patent is:
1. Method of coloring a material containing an  
 65 organic derivative of cellulose comprising applying  
 thereto a composition containing a dyestuff  
 having substantially no affinity for the organic  
 derivative of cellulose and a volatile organic  
 liquid having at least a softening action on said  
 70 organic derivative of cellulose and having a boiling  
 point of over 100° C. and then drying.
2. Method of coloring a material containing cellulose acetate comprising applying thereto a composition containing a dyestuff having substantially no affinity for the cellulose acetate and a volatile organic liquid having at least a softening action on said cellulose acetate and having a boiling point of over 100° C. and then drying. 80
3. Method of coloring a material containing cellulose acetate comprising applying thereto a composition containing a dyestuff having substantially no affinity for the organic derivative of cellulose and a large amount of a volatile organic liquid having at least a softening action on said cellulose acetate and having a boiling point above 100° C. and then drying. 85
4. Method of coloring a material containing cellulose acetate comprising applying thereto a composition containing a dyestuff having substantially no affinity for the cellulose acetate and ethyl lactate and then drying. 90
5. Method of coloring a material containing an organic derivative of cellulose comprising applying thereto a composition containing a dyestuff having substantially no affinity for the organic derivative of cellulose when applied in simple dyebaths and a large amount of a volatile organic liquid having at least a softening action on said organic derivative of cellulose and having a boiling point of over 100° C. and then drying. 95
6. Method of coloring a material containing cellulose acetate comprising applying thereto a composition containing a dyestuff having substantially no affinity for the cellulose acetate when applied in simple dyebaths and a large amount of a volatile organic liquid having at least a softening action on said cellulose acetate and having a boiling point of over 100° C. and then drying. 100
7. Method of locally coloring a textile material containing an organic derivative of cellulose yarn comprising locally applying thereto a printing paste containing a dyestuff having substantially no affinity for the organic derivative of cellulose and a large amount of a volatile organic liquid having a boiling point above 100° C. and which exerts at least a softening action on the organic derivative of cellulose and then quickly drying below 100° C. 105
8. Method of locally coloring a textile material containing cellulose acetate comprising locally applying thereto a printing paste containing a dyestuff having substantially no affinity for the cellulose acetate and a large amount of a volatile organic liquid having a boiling point above 100° C. and which exerts at least a softening action on the cellulose acetate and then quickly drying below 100° C. 110
9. Method of producing differential lustre and color effects on a fabric containing cellulose acetate yarn comprising locally applying to a de-lustered cellulose acetate fabric a printing paste comprising a dyestuff having substantially no affinity for the cellulose acetate and a volatile organic liquid having a boiling point above 100° C. and which exerts at least a softening action on the cellulose acetate and then drying below 100° C. 115

GEORGE RIVAT.

145